



US010806970B2

(12) **United States Patent**  
**Bulpett et al.**

(10) **Patent No.:** **US 10,806,970 B2**  
(45) **Date of Patent:** **Oct. 20, 2020**

(54) **GOLF BALL COMPOSITIONS**

(71) Applicant: **Acushnet Company**, Fairhaven, MA (US)

(72) Inventors: **David A. Bulpett**, Boston, MA (US); **Brian Comeau**, Berkley, MA (US); **Michael J. Sullivan**, Old Lyme, CT (US); **Mark L. Binette**, Mattapoisett, MA (US); **Robert Blink**, Newport, RI (US)

(73) Assignee: **Acushnet Company**, Fairhaven, MA (US)

(\*) Notice: Subject to any disclaimer, the term of this patent is extended or adjusted under 35 U.S.C. 154(b) by 0 days.

(21) Appl. No.: **16/042,138**

(22) Filed: **Jul. 23, 2018**

(65) **Prior Publication Data**

US 2018/0339200 A1 Nov. 29, 2018

**Related U.S. Application Data**

(62) Division of application No. 13/849,576, filed on Mar. 25, 2013, now Pat. No. 10,035,045.

(51) **Int. Cl.**

**A63B 37/06** (2006.01)

**A63B 37/00** (2006.01)

(52) **U.S. Cl.**

CPC ..... **A63B 37/0074** (2013.01); **A63B 37/0039** (2013.01); **A63B 37/0073** (2013.01)

(58) **Field of Classification Search**

CPC ..... A63B 37/0077

USPC ..... 473/351

See application file for complete search history.

(56) **References Cited**

**U.S. PATENT DOCUMENTS**

|                   |         |                     |              |
|-------------------|---------|---------------------|--------------|
| 5,050,886 A *     | 9/1991  | Yamagishi .....     | A63B 37/0003 |
|                   |         |                     | 473/372      |
| 5,733,974 A       | 3/1998  | Yamada et al.       |              |
| 5,779,561 A       | 7/1998  | Sullivan et al.     |              |
| 5,789,486 A       | 8/1998  | Maruoka et al.      |              |
| 6,186,906 B1      | 2/2001  | Sullivan et al.     |              |
| 6,361,453 B1      | 3/2002  | Nakamura et al.     |              |
| 6,465,573 B1      | 10/2002 | Maruko et al.       |              |
| 7,182,700 B2      | 2/2007  | Endo et al.         |              |
| 7,402,114 B2      | 7/2008  | Binette et al.      |              |
| 7,612,135 B2      | 11/2009 | Kennedy, III et al. |              |
| 9,044,644 B2      | 6/2015  | Shinohara           |              |
| 2003/0148826 A1 * | 8/2003  | Ohama .....         | A63B 37/0003 |
|                   |         |                     | 473/371      |
| 2003/0216520 A1   | 11/2003 | Irii et al.         |              |
| 2008/0234070 A1   | 9/2008  | Comeau et al.       |              |
| 2010/0331109 A1   | 12/2010 | Sullivan et al.     |              |
| 2012/0165122 A1   | 6/2012  | Kim et al.          |              |

\* cited by examiner

*Primary Examiner* — Raeann Gorden

(74) *Attorney, Agent, or Firm* — Mandi B. Milbank

(57) **ABSTRACT**

Disclosed herein are heterogeneous golf ball compositions comprising a matrix formed from a thermosetting polymer composition and discrete particles of crosslinked rubber dispersed within the matrix.

**7 Claims, No Drawings**

## 1

## GOLF BALL COMPOSITIONS

CROSS-REFERENCE TO RELATED  
APPLICATIONS

The present application is a division of U.S. patent application Ser. No. 13/849,576, filed Mar. 25, 2013, the entire disclosure of which is hereby incorporated herein by reference.

## FIELD OF THE INVENTION

The present invention is directed to golf ball compositions comprising discrete particles of crosslinked rubber within a thermosetting polymer matrix.

## BACKGROUND OF THE INVENTION

U.S. Pat. No. 5,789,486 to Maruoka et al. discloses a golf ball including a paint layer comprised of a dispersion of internally-crosslinked polymer gel fine particles.

U.S. Pat. No. 6,186,906 to Sullivan et al. discloses golf ball compositions comprising discrete particles of gel.

U.S. Pat. No. 7,402,114 to Binette et al. discloses golf ball materials comprising a partially to highly neutralized blend of copolymers, a fatty acid or fatty acid salt, and a heavy mass filler.

U.S. Pat. No. 7,612,135 to Kennedy, III et al. discloses golf ball materials comprising a partially to highly neutralized blend of an acid copolymer, a copolymer comprising a metallocene-catalyzed alpha-olefin and a softening comonomer, and a fatty acid or fatty acid salt.

U.S. Patent Application Publication No. 2008/0234070 to Comeau et al. discloses the use of crosslinked rubber nanoparticles in golf ball layers.

U.S. Pat. No. 5,733,974 to Yamada et al. discloses a golf ball comprising a core made of an elastomer and a cover covering said core wherein said cover is made of a thermoplastic material comprising a rubber powder and a thermoplastic elastomer.

U.S. Pat. No. 6,465,573 to Maruko et al. discloses a solid golf ball comprising a core, an intermediate layer, and a cover improved in rebound, distance, and feel when the intermediate layer is comprised of a thermoplastic resin in admixture with rubber powder.

U.S. Pat. No. 5,779,561 to Sullivan et al. discloses a golf ball including an inner cover layer comprising (1) a first resin composition containing at least 50 parts by weight of a non-ionomer polyolefin material and (2) at least one part by weight of a filler.

U.S. Patent Application Publication No. 2003/0216520 to Irii et al. discloses a golf ball whose core is covered with a cover, wherein the core is constituted of a rubber composition containing polybutadiene rubber and the cover is constituted of a resin composition composed of ionomer resin and diene rubber.

U.S. Patent Application Publication No. 2012/0165122 to Kim et al. discloses a golf ball where at least one of the outer cover layer and the intermediate layer includes a blend composition of about 2 to about 40 wt % of a polyamide and about 60 to about 98 wt % of one or more of either a block copolymer, an acidic copolymer; an acidic terpolymer; an ionomer, or a multi component blend composition; and wherein the polyamide has a melting point which is greater than about 5 and less than about 200° C. above the melting point of the other blend component.

## 2

U.S. Pat. No. 6,361,453 to Nakamura et al. discloses a solid golf ball having a solid core and a cover, the solid core is composed of a core-forming material and particles of a different material.

5

## SUMMARY OF THE INVENTION

The present invention is directed to a golf ball comprising a layer formed from a heterogeneous composition, the composition comprising a matrix formed from a thermosetting polymer composition and discrete particles dispersed within the matrix.

In a particular embodiment, the discrete particles are formed from a crosslinked rubber composition having a Shore D hardness of 65 or greater.

In another particular embodiment, the discrete particles are formed from a crosslinked rubber composition having a Shore C hardness of 40 or less.

In another particular embodiment, the discrete particles are formed from a crosslinked rubber composition comprising a peroxide initiator and 50 phr or greater of a coagent.

In another particular embodiment, the discrete particles are formed from a sulfur-cured diene rubber composition.

In another particular embodiment, the discrete particles are formed from a crosslinked rubber composition comprising a peroxide initiator and from 0 to 5 phr of a coagent.

In another particular embodiment, the thermosetting matrix composition comprises a base rubber selected from ethylene propylene rubbers, ethylene-propylene-diene rubbers, styrene-butadiene rubbers, butyl rubbers, halobutyl rubbers, acrylonitrile butadiene rubbers, polychloroprenes, alkyl acrylate rubbers, chlorinated isoprene rubbers, acrylonitrile chlorinated isoprene rubbers, polyalkenamers, phenol formaldehydes, melamine formaldehydes, polyepoxides, polyimides, polysiloxanes, alkyds, polyisocyanurates, poly-cyanurates, polyacrylates, and combinations of two or more thereof.

## DETAILED DESCRIPTION

Golf ball compositions of the present invention are heterogeneous compositions comprising discrete particles of crosslinked material within a matrix formed from a thermosetting polymer composition. The heterogeneous composition is formed by adding the particles to the matrix composition either prior to or during the process of forming the golf ball layer.

In a particular embodiment, the heterogeneous composition has a solid sphere coefficient of restitution, "COR," within a range having a lower limit of 0.450 or 0.500 or 0.550 or 0.600 or 0.650 or 0.700 and an upper limit of 0.710 or 0.730 or 0.750 or 0.770 or 0.800 or 0.820 or 0.850 or 0.870 or 0.900 or 0.910 or 0.930. For purposes of the present disclosure, the "solid sphere COR" of a composition refers to the COR of a cured 1.55 inch diameter sphere of the composition. COR is determined according to a known procedure wherein a sphere is fired from an air cannon at two given velocities and calculated at a velocity of 125 ft/s. Ballistic light screens are located between the air cannon and the steel plate at a fixed distance to measure ball velocity. As the sphere travels toward the steel plate, it activates each light screen, and the time at each light screen is measured. This provides an incoming transit time period inversely proportional to the sphere's incoming velocity. The sphere impacts the steel plate and rebounds through the light screens, which again measures the time period required to transit between the light screens. This provides an outgoing

transit time period inversely proportional to the sphere's outgoing velocity. COR is then calculated as the ratio of the outgoing transit time period to the incoming transit time period,  $COR = V_{out}/V_{in} = T_{in}/T_{out}$ .

In a particular embodiment, the heterogeneous composition has a solid sphere compression within a range having a lower limit of -75 or -50 or -20 or 0 or 10 or 15 and an upper limit of 20 or 25 or 30 or 35 or 40 or 50. In another particular embodiment, the heterogeneous composition has a solid sphere compression within a range having a lower limit of 70 or 75 or 80 or 85 or 90 and an upper limit of 90 or 95 or 100 or 105 or 115 or 120 or 125. In another particular embodiment, the heterogeneous composition has a solid sphere compression within a range having a lower limit of 120 or 130 or 140 or 150 or 155 or 160 and an upper limit of 160 or 165 or 170 or 180 or 190 or 200. In another particular embodiment, the heterogeneous composition has a solid sphere compression of 130 or greater, or 140 or greater, or 150 or greater, or 155 or greater, or 160 or greater, or 165 or greater, or 170 or greater. For purposes of the present disclosure, the "solid sphere compression" of a composition refers to the compression of a cured 1.55 inch diameter sphere of the composition. The compression of the sphere is determined according to a known procedure, using a digital Atti compression test device, wherein a piston is used to compress a sphere against a spring. Conversion from Atti compression to Riehle (cores), Riehle (balls), 100 kg deflection, 130-10 kg deflection or effective modulus can be carried out according to the formulas given in Jeff Dalton's *Compression by Any Other Name, Science and Golf IV, Proceedings of the World Scientific Congress of Golf* (Eric Thain ed., Routledge, 2002).

In a particular embodiment, the heterogeneous composition has a flexural modulus of 5 ksi or greater, 6 ksi or greater, or 8 ksi or greater, or 10 ksi or greater, or 15 ksi or greater, or 20 ksi or greater, or 25 ksi or greater, or 30 ksi or greater, or 35 ksi or greater, or 40 ksi or greater, or 45 ksi or greater, or 48 ksi or greater, or 50 ksi or greater, or 52 ksi or greater, or 55 ksi or greater, or 60 ksi or greater, or 63 ksi or greater, or 65 ksi or greater, or 70 ksi or greater, 100 ksi or greater, or 120 ksi or greater, or 150 ksi or greater, or 160 ksi or greater, or 170 ksi or greater, or 180 ksi or greater, or 195 ksi or greater, or a flexural modulus within a range having a lower limit of 5 or 6 or 8 or 10 or 15 or 20 or 25 or 30 or 35 or 40 or 45 or 48 or 50 or 52 or 55 or 56 or 60 or 63 or 65 or 70 ksi and an upper limit of 75 or 80 or 85 or 90 or 95 or 100 or 105 or 110 or 115 ksi, or a flexural modulus within a range having a lower limit of 20 or 25 or 30 or 35 or 40 or 45 or 50 or 55 or 60 ksi and an upper limit of 60 or 65 or 70 or 75 or 80 ksi, or a flexural modulus within a range having a lower limit of 50 or 60 or 70 or 90 or 120 or 130 and an upper limit of 150 or 170 or 200 or 210. For purposes of the present disclosure, flex modulus is measured according to the following procedure. Flex bars are prepared by compression molding the composition under sufficient temperature and pressure for a sufficient amount of time to produce void- and defect-free plaques of appropriate dimensions to produce the required flex bars. The flex bar dimensions are about 0.125 inches by about 0.5 inches, and of a length sufficient to satisfy the test requirements. Flex bars are die cut from the compression molded plaque(s) soon after the blend composition has reached room temperature. The flex bars are then aged for 14 days at 23° C. and 50% RH before testing. Flex modulus is then measured according to ASTM D790 Procedure B, using a load span of 1.0 inches, a support span length of 2.0 inches, a support span-to-depth

ratio of 16:1 and a crosshead rate of 0.5 inches/minute. The support and loading noses have a radius of 5 mm.

In a particular embodiment, the particles are present in the composition in an amount of 1 wt % or greater, or 2 wt % or greater, or 3 wt % or greater, or 5 wt % or greater, or 10 wt % or greater, or 15 wt % or greater, or 18 wt % or greater, or 20 wt % or greater, or 25 wt % or greater, or 30 wt % or greater, or 35 wt % or greater, or 40 wt % or greater, or 45 wt % or greater, or 50 wt % or greater, or 55 wt % or greater, or 60 wt % or greater, or an amount within a range having a lower limit of 1 or 2 or 3 or 5 or 10 or 15 or 20 or 25 or 30 or 35 or 40 wt % and an upper limit of 50 or 55 or 60 or 65 or 70 or 75 or 80 or 85 or 90 wt %, based on the total weight of the composition.

In another particular embodiment, the composition comprises at least 500 of the discrete particles.

In a particular embodiment, the particles have a maximum particle size of 0.595 mm or 0.707 mm or 0.841 mm or 0.900 mm or 1.00 mm or 1.19 mm or 1.41 mm or 1.68 mm or 2.00 mm or 2.38 mm. In another embodiment, the crosslinked particles have a particle size within a range having a lower limit of 0.001 mm or 0.002 mm or 0.005 mm or 0.007 mm or 0.015 mm or 0.030 mm or 0.037 mm or 0.074 mm and an upper limit of 0.100 mm or 0.125 mm or 0.177 mm or 0.354 mm or 0.420 mm or 0.500 mm or 0.595 mm or 0.707 mm or 0.841 mm or 1.000 mm or 1.19 mm or 1.41 mm or 1.68 mm or 2.00 mm or 2.38 mm.

#### Particle Composition

For purposes of the present invention, the particle composition is crosslinked and ground into particles prior to being added to the matrix composition.

Rubber compositions suitable for forming the particles include a base rubber selected from natural rubber, polybutadiene, polyisoprene, ethylene propylene rubber (EPR), ethylene-propylene-diene rubber (EPDM), styrene-butadiene rubber, butyl rubber, halobutyl rubber, polyurethane, polyurea, acrylonitrile butadiene rubber, polychloroprene, alkyl acrylate rubber, chlorinated isoprene rubber, acrylonitrile chlorinated isoprene rubber, polyalkenamer, phenol formaldehyde, melamine formaldehyde, polyepoxide, polysiloxane, polyester, alkyd, polyisocyanurate, polycyanurate, polyacrylate, and combinations of two or more thereof. Diene rubbers are preferred, particularly polybutadiene, styrene-butadiene, acrylonitrile butadiene, and mixtures of polybutadiene with other elastomers wherein the amount of polybutadiene present is at least 40 wt % based on the total polymeric weight of the mixture.

Non-limiting examples of suitable commercially available rubbers are Buna CB high-cis neodymium-catalyzed polybutadiene rubbers, such as Buna CB 23, and Buna CB high-cis cobalt-catalyzed polybutadiene rubbers, such as Buna CB 1220 and 1221, commercially available from Lanxess Corporation; SE BR-1220, commercially available from The Dow Chemical Company; Europrene® NEOCIS® 55 BR 40 and BR 60, commercially available from Polimeri Europa®, UBEPOL-BR® rubbers, commercially available from UBE Industries, Inc.; BR 01, commercially available from Japan Synthetic Rubber Co., Ltd.; Neodene high-cis neodymium-catalyzed polybutadiene rubbers, such as Neodene BR 40, commercially available from Karbochem; TP-301 transpolyisoprene, commercially available from Kuraray Co., Ltd.; Vestenamer® polyoctenamer, commercially available from Evonik Industries; Butyl 065 and Butyl 288 butyl rubbers, commercially available from ExxonMobil Chemical Company; Butyl 301 and Butyl 101-3, commercially available from Lanxess Corporation; Bromobutyl 2224 and Chlorobutyl 1066 halobutyl rubbers, commercially

available from ExxonMobil Chemical Company; Bromobutyl X2 and Chlorobutyl 1240 halobutyl rubbers, commercially available from Lanxess Corporation; BromoButyl 2255 butyl rubber, commercially available from Japan Synthetic Rubber Co., Ltd.; Vistalon® 404 and Vistalon® 706 ethylene propylene rubbers, commercially available from ExxonMobil Chemical Company; Dutral CO 058 ethylene propylene rubber, commercially available from Polimeri Europa; Nordel® IP NDR 5565 and Nordel® IP 3670 ethylene-propylene-diene rubbers, commercially available from The Dow Chemical Company; EPT1045 and EPT1045 ethylene-propylene-diene rubbers, commercially available from Mitsui Corporation; Buna SE 1721 TE styrene-butadiene rubbers, commercially available from Lanxess Corporation; Afpol 1500 and Afpol 552 styrene-butadiene rubbers, commercially available from Karbochem; Nipol® DN407 and Nipol® 1041L acrylonitrile butadiene rubbers, commercially available from Zeon Chemicals, L.P.; Neoprene GRT and Neoprene AD30 polychloroprene rubbers; Vamac® ethylene acrylic elastomers, commercially available from E. I. du Pont de Nemours and Company; Hytemp® AR12 and AR214 alkyl acrylate rubbers, commercially available from Zeon Chemicals, L.P.; and Hypalon® chlorosulfonated polyethylene rubbers, commercially available from E. I. du Pont de Nemours and Company.

The rubber is crosslinked using, for example, a peroxide or sulfur cure system, C—C initiators, high energy radiation sources capable of generating free radicals, or a combination thereof.

In a particular embodiment, the rubber is crosslinked using a peroxide initiator and optionally a coagent. Suitable peroxide initiators include, but are not limited to, organic peroxides, such as dicumyl peroxide; n-butyl-4,4-di(t-butylperoxy) valerate; 1,1-di(t-butylperoxy)3,3,5-trimethylcyclohexane; 2,5-dimethyl-2,5-di(t-butylperoxy) hexane; di-t-butyl peroxide; di-t-amyl peroxide; t-butyl peroxide; t-butyl cumyl peroxide; 2,5-dimethyl-2,5-di(t-butylperoxy)hexyne-3; di(2-t-butyl-peroxyisopropyl)benzene; dilauroyl peroxide; dibenzoyl peroxide; t-butyl hydroperoxide; lauryl peroxide; benzoyl peroxide; and combinations thereof. Examples of suitable commercially available peroxides include, but are not limited to Perkadox® BC dicumyl peroxide, commercially available from Akzo Nobel, and Varox® peroxides, such as Varox® ANS benzoyl peroxide and Varox® 231 1,1-di(t-butylperoxy)3,3,5-trimethylcyclohexane, commercially available from RT Vanderbilt Company, Inc.

Coagents are commonly used with peroxides to increase the state of cure. Suitable coagents include, but are not limited to, metal salts of unsaturated carboxylic acids; unsaturated vinyl compounds and polyfunctional monomers (e.g., trimethylolpropane trimethacrylate); maleimides (e.g., phenylene bismaleimide); and combinations thereof. Particular examples of suitable metal salts of unsaturated carboxylic acids include, but are not limited to, one or more metal salts of acrylates, diacrylates, methacrylates, and dimethacrylates, wherein the metal is selected from magnesium, calcium, zinc, aluminum, lithium, nickel, and sodium. In a particular embodiment, the coagent is selected from zinc salts of acrylates, diacrylates, methacrylates, dimethacrylates, and mixtures thereof. In another particular embodiment, the coagent is zinc diacrylate.

The amount of peroxide initiator and coagent can be varied to achieve the desired hardness of the crosslinked particle composition. For example, in one embodiment, the crosslinked particle composition is a coagent-cured rubber comprising a peroxide initiator and a high level of coagent

(e.g., 35 phr or greater, or greater than 35 phr, or 50 phr or greater, or greater than 50 phr, or 75 phr or greater, or greater than 75 phr of coagent, or 100 phr or greater, or 150 hr or greater, or 200 phr or greater, or 250 phr or greater, or 300 phr or greater, or 350 phr or greater, or 400 phr or greater). In a particular aspect of this embodiment, the crosslinked particle composition has a Shore D hardness of 55 or greater, or greater than 55, or 60 or greater, or greater than 60, or 65 or greater, or greater than 65, or 70 or greater, or greater than 70, or 75 or greater, or greater than 75, or 80 or greater, or greater than 80, or 85 or greater, or greater than 85, or 90 or greater, or greater than 90. In another embodiment, the crosslinked particle composition is a peroxide-cured rubber comprising a peroxide initiator and is free of coagent, substantially free of coagent (i.e., <1 phr coagent), or includes a low level of coagent (e.g., 10 phr or less, or less than 10 phr, or 5 phr or less, or less than 5 phr, or 1 phr or less, or less than 1 phr). In a particular aspect of this embodiment, the crosslinked particle composition has a Shore C hardness of 50 or less, or less than 50, or 45 or less, or less than 45, or 40 or less, or less than 40, or 35 or less, or less than 35, or 30 or less, or less than 30, or 25 or less, or less than 25, or 20 or less, or less than 20, or 15 or less, or 12 or less, or 10 or less, or a Shore A hardness of 55 or less, or less than 55, or 50 or less, or less than 50, or 40 or less, or 30 or less. In another embodiment, the crosslinked particle composition is a peroxide-cured rubber comprising a peroxide initiator and a coagent, wherein the peroxide initiator is present in an amount of at least 0.05 phr, or an amount within a range having a lower limit of 0.05 or 0.1 or 0.8 or 1 or 1.25 or 1.5 phr and an upper limit of 2.5 or 3 or 5 or 6 or 10 or 15 phr, and wherein the coagent is present in an amount within a range having a lower limit of 1 or 5 or 10 or 15 or 19 or 20 phr and an upper limit of 24 or 25 or 30 or 35 or 40 or 45 or 50 or 60 phr. In a particular aspect of this embodiment, the crosslinked particle composition has a Shore C hardness within a range having a lower limit of 20 or 25 or 30 or 35 or 40 or 45 or 50 or 55 or 60 or 70 or 80 or 82 or 85 and an upper limit of 60 or 70 or 75 or 80 or 90 or 92 or 93 or 95, wherein the upper limit is greater than the lower limit (e.g., when the lower limit is 70, the upper limit is 75, 80, 90, 92, 93, or 95).

In another particular embodiment, the rubber is crosslinked using sulfur and/or an accelerator. Suitable accelerators include, but are not limited to, guanidines (e.g., diphenyl guanidine, triphenyl guanidine, and di-ortho-tolyl guanidine); thiazoles (e.g., mercaptobenzothiazole, dibenzothiazyl disulfide, sodium salt of mercaptobenzothiazole, zinc salt of mercaptobenzothiazole, and 2,4-dinitrophenyl mercaptobenzothiazole); sulfenamides (e.g., N-cyclohexylbenzothiazylsulfenamide, N-oxydiethylbenzothiazylsulfenamide, N-t-butylbenzothiazylsulfenamide, and N,N'-dicyclohexylbenzothiazylsulfenamide); thiuram sulfides (e.g., tetramethyl thiuram disulfide, tetraethyl thiuram disulfide, tetrabutylthiuram disulfide, tetramethyl thiuram monosulfide, dipentamethylene thiuram tetrasulfate, 4-morpholiny-2-benzothiazole disulfide, and dipentamethylenethiuram hexa-sulfide); dithiocarbamates (e.g., piperidine pentamethylene dithiocarbamate, zinc diethyl dithiocarbamate, sodium diethyl dithiocarbamate, zinc ethyl phenyl dithiocarbamate, and bismuth dimethyl dithiocarbamate); thioureas (e.g., ethylene thiourea, N,N'-diethylthiourea, and N,N'-diphenylthiourea); xanthates (e.g., zinc isopropyl xanthate, sodium isopropyl xanthate, and zinc butyl xanthate); dithiophosphates; and aldehyde amines (e.g., hexamethylene tetramine and ethylidene aniline).

The crosslinking system optionally includes one or more activators selected from metal oxides (e.g., zinc oxide and magnesium oxide), and fatty acids and salts of fatty acids (e.g., stearic acid, zinc stearate, oleic acid, and dibutyl ammonium oleate).

The rubber particle composition optionally includes a scorch retarder to prevent scorching of the rubber during processing before vulcanization. Suitable scorch retarders include, but are not limited to, salicylic acid, benzoic acid, acetylsalicylic acid, phthalic anhydride, sodium acetate, and N-cyclohexylthiophthalimide.

The rubber particle composition optionally includes one or more antioxidants to inhibit or prevent the oxidative degradation of the base rubber. Some antioxidants also act as free radical scavengers; thus, when antioxidants are included in the crosslinked particle composition, the amount of initiator agent used may be as high as or higher than the amounts disclosed herein. Suitable antioxidants include, but are not limited to, hydroquinoline antioxidants, phenolic antioxidants, and amine antioxidants.

The rubber particle composition optionally includes from 0.05 phr to 10.0 phr of a soft and fast agent selected from organosulfur and metal-containing organosulfur compounds; organic sulfur compounds, including mono, di, and polysulfides, thiol, and mercapto compounds; inorganic sulfide compounds; blends of an organosulfur compound and an inorganic sulfide compound; Group VIA compounds; substituted and unsubstituted aromatic organic compounds that do not contain sulfur or metal; aromatic organometallic compounds; hydroquinones; benzoquinones; quinhydrones; catechols; resorcinols; and combinations thereof. In a particular embodiment, the soft and fast agent is selected from zinc pentachlorothiophenol, pentachlorothiophenol, ditolyl disulfide, diphenyl disulfide, dixylyl disulfide, 2-nitroresorcinol, and combinations thereof.

The rubber particle composition optionally contains one or more fillers. Exemplary fillers include precipitated hydrated silica, clay, talc, asbestos, glass fibers, aramid fibers, mica, calcium metasilicate, zinc sulfate, barium sulfate, zinc sulfide, lithopone, silicates, silicon carbide, diatomaceous earth, carbonates (e.g., calcium carbonate, zinc carbonate, barium carbonate, and magnesium carbonate), metals (e.g., titanium, tungsten, aluminum, bismuth, nickel, molybdenum, iron, lead, copper, boron, cobalt, beryllium, zinc, and tin), metal alloys (e.g., steel, brass, bronze, boron carbide whiskers, and tungsten carbide whiskers), oxides (e.g., zinc oxide, tin oxide, iron oxide, calcium oxide, aluminum oxide, titanium dioxide, magnesium oxide, and zirconium oxide), particulate carbonaceous materials (e.g., graphite, carbon black, cotton flock, natural bitumen, cellulose flock, and leather fiber), microballoons (e.g., glass and ceramic), fly ash, core material that is ground and recycled, nanofillers and combinations thereof. The amount of particulate material(s) present in the rubber particle composition is typically within a range having a lower limit of 5 parts or 10 parts by weight per 100 parts of the base polymer, and an upper limit of 30 parts or 50 parts or 100 parts by weight per 100 parts of the base polymer. Filler materials may be dual-functional fillers, such as zinc oxide (which may be used as a filler/acid scavenger) and titanium dioxide (which may be used as a filler/brightener material).

The rubber particle composition may also contain one or more additives selected from processing aids, such as trans-polyisoprene (e.g., TP-301 transpolyisoprene, commercially available from Kuraray Co., Ltd.), transbutadiene rubber, and polyalkenamer rubber; processing oils; plasticizers; coloring agents; fluorescent agents; chemical blowing and

foaming agents; defoaming agents; stabilizers; softening agents; impact modifiers; free radical scavengers; antioxidants (e.g., p-phenylenediamines); and the like. The amount of additive(s) typically present in the crosslinked particle composition is typically within a range having a lower limit of 0 parts or 5 parts by weight per 100 parts of the base polymer, and an upper limit of 10 parts or 20 parts or 50 parts or 100 parts or 150 parts by weight per 100 parts of the base polymer.

10 Suitable types and amounts of rubber, initiator agent, coagent, filler, and additives are more fully described in, for example, U.S. Pat. Nos. 6,566,483, 6,695,718, 6,939,907, 7,041,721 and 7,138,460, the entire disclosures of which are hereby incorporated herein by reference. Particularly suitable diene rubber compositions are further disclosed, for example, in U.S. Patent Application Publication No. 2007/0093318, the entire disclosure of which is hereby incorporated herein by reference.

In a particular embodiment, the crosslinked rubber particle composition has a Shore D hardness of 55 or greater, or greater than 55, or 60 or greater, or greater than 60, or 65 or greater, or greater than 65, or 70 or greater, or greater than 70, or 75 or greater, or greater than 75, or 80 or greater, or greater than 80, or 85 or greater, or greater than 85, or 90 or greater, or greater than 90.

In another particular embodiment, the crosslinked rubber particle composition has a Shore C hardness of 50 or less, or less than 50, or 45 or less, or less than 45, or 40 or less, or less than 40, or 35 or less, or less than 35, or 30 or less, or less than 30, or 25 or less, or less than 25, or 20 or less, or less than 20, or 15 or less, or 12 or less, or 10 or less.

In another particular embodiment, the crosslinked rubber particle composition has a Shore A hardness of 55 or less, or less than 55, or 50 or less, or less than 50, or 40 or less, or less than 30 or less.

In another particular embodiment, the crosslinked rubber particle composition has a Shore C hardness within a range having a lower limit of 20 or 25 or 30 or 35 or 40 or 45 or 50 or 55 or 60 or 70 or 80 or 82 or 85 and an upper limit of 60 or 70 or 75 or 80 or 90 or 92 or 93 or 95, wherein the upper limit is greater than the lower limit (e.g., when the lower limit is 70, the upper limit is 75, 80, 90, 92, 93, or 95).

For purposes of the present disclosure, the hardness of the crosslinked rubber particle composition refers to the surface hardness of a 0.25 inch plaque of the composition cured under the same conditions as those used to cure the particle composition that is added to the matrix composition to form the heterogeneous composition. Hardness measurements are made pursuant to ASTM D-2240 using a calibrated, digital durometer, capable of reading to 0.1 hardness units and set to record the maximum hardness reading obtained for each measurement.

#### Matrix Composition

Thermosetting compositions suitable for forming the matrix include a base rubber selected from natural rubbers, polybutadienes, polyisoprenes, ethylene propylene rubbers (EPR), ethylene-propylene-diene rubbers (EPDM), styrene-butadiene rubbers, butyl rubbers, halobutyl rubbers, polyurethanes, polyureas, acrylonitrile butadiene rubbers, poly-chloroprenes, alkyl acrylate rubbers, chlorinated isoprene rubbers, polyalkenamers, phenol formaldehydes, melamine formaldehydes, polyepoxides, polysiloxanes, polyesters, alkyds, polyisocyanurates, polycyanurates, polyacrylates, and combinations of two or more thereof.

65 Non-limiting examples of suitable commercially available thermosetting materials are Buna CB high-cis neodymium-catalyzed polybutadiene rubbers, such as Buna CB

23, and Buna CB high-cis cobalt-catalyzed polybutadiene rubbers, such as Buna CB 1220 and 1221, commercially available from Lanxess Corporation; SE BR-1220, commercially available from The Dow Chemical Company; Europrene® NEOCIS® BR 40 and BR 60, commercially available from Polimeri Europa®; UBEPOL-BR® rubbers, commercially available from UBE Industries, Inc.; BR 01, commercially available from Japan Synthetic Rubber Co., Ltd.; Neodene high-cis neodymium-catalyzed polybutadiene rubbers, such as Neodene BR 40, commercially available from Karbochem; TP-301 transpolyisoprene, commercially available from Kuraray Co., Ltd.; Vestenamer® polyoctenamer, commercially available from Evonik Industries; Butyl 065 and Butyl 288 butyl rubbers, commercially available from ExxonMobil Chemical Company; Butyl 301 and Butyl 101-3, commercially available from Lanxess Corporation; Bromobutyl 2224 and Chlorobutyl 1066 halobutyl rubbers, commercially available from ExxonMobil Chemical Company; Bromobutyl X2 and Chlorobutyl 1240 halobutyl rubbers, commercially available from Lanxess Corporation; BromoButyl 2255 butyl rubber, commercially available from Japan Synthetic Rubber Co., Ltd.; Vistalon® 404 and Vistalon® 706 ethylene propylene rubbers, commercially available from ExxonMobil Chemical Company; Dutral Colo. 058 ethylene propylene rubber, commercially available from Polimeri Europa; Nordel® IP NDR 5565 and Nordel® IP 3670 ethylene-propylene-diene rubbers, commercially available from The Dow Chemical Company; EPT1045 and EPT1045 ethylene-propylene-diene rubbers, commercially available from Mitsui Corporation; Buna SE 1721 TE styrene-butadiene rubbers, commercially available from Lanxess Corporation; Afpol 1500 and Afpol 552 styrene-butadiene rubbers, commercially available from Karbochem; Nipol® DN407 and Nipol® 1041L acrylonitrile butadiene rubbers, commercially available from Zeon Chemicals, L.P.; Neoprene GRT and Neoprene AD30 polychloroprene rubbers; Vamac® ethylene acrylic elastomers, commercially available from E. I. du Pont de Nemours and Company; Hytemp® AR12 and AR214 alkyl acrylate rubbers, commercially available from Zeon Chemicals, L.P.; and Hypalon® chlorosulfonated polyethylene rubbers, commercially available from E. I. du Pont de Nemours and Company.

The matrix composition may contain one or more fillers. Exemplary fillers include precipitated hydrated silica, clay, talc, asbestos, glass fibers, aramid fibers, mica, calcium metasilicate, zinc sulfate, barium sulfate, zinc sulfide, lithopone, silicates, silicon carbide, diatomaceous earth, carbonates (e.g., calcium carbonate, zinc carbonate, barium carbonate, and magnesium carbonate), metals (e.g., titanium, tungsten, aluminum, bismuth, nickel, molybdenum, iron, lead, copper, boron, cobalt, beryllium, zinc, and tin), metal alloys (e.g., steel, brass, bronze, boron carbide whiskers, and tungsten carbide whiskers), oxides (e.g., zinc oxide, tin oxide, iron oxide, calcium oxide, aluminum oxide, titanium dioxide, magnesium oxide, and zirconium oxide), particulate carbonaceous materials (e.g., graphite, carbon black, cotton flock, natural bitumen, cellulose flock, and leather fiber), microballoons (e.g., glass and ceramic), fly ash, core material that is ground and recycled, nanofillers and combinations thereof.

The matrix composition may also contain one or more additives selected from processing aids, such as transpolyisoprene (e.g., TP-301 transpolyisoprene, commercially available from Kuraray Co., Ltd.), transbutadiene rubber, and polyalkenamer rubber; processing oils; plasticizers; coloring agents; fluorescent agents; chemical blowing and

foaming agents; defoaming agents; stabilizers; softening agents; impact modifiers; free radical scavengers; accelerators; scorch retarders; antiozonants (e.g., p-phenylenediamines); and the like.

5 The matrix composition may also contain one or more antioxidants. Antioxidants are compounds that can inhibit or prevent the oxidative degradation of the rubber. Some antioxidants also act as free radical scavengers; thus, when antioxidants are included in the rubber composition, the amount of initiator agent used may be as high as or higher than the amounts disclosed herein. Suitable antioxidants include, for example, hydroquinoline antioxidants, phenolic antioxidants, and amine antioxidants.

10 Suitable rubbers are more fully described in, for example, U.S. Pat. Nos. 6,566,483, 6,695,718, 6,939,907, 7,041,721 and 7,138,460, the entire disclosures of which are hereby incorporated herein by reference. Particularly suitable diene rubber compositions are further disclosed, for example, in U.S. Patent Application Publication No. 2007/0093318, the entire disclosure of which is hereby incorporated herein by reference.

#### Golf Ball Applications

15 Golf ball compositions according to the present invention can be used in a variety of constructions. For example, the compositions are suitable for use in one-piece, two-piece (i.e., a core and a cover), multi-layer (i.e., a core of one or more layers and a cover of one or more layers), and wound golf balls, having a variety of core structures, intermediate layers, covers, and coatings.

20 In golf balls of the present invention, at least one layer comprises a heterogeneous composition comprising discrete particles of crosslinked material within a thermosetting polymer matrix, as described herein. In golf balls having two or more layers comprising a composition of the present invention, the inventive composition of one layer may be the same as or a different inventive composition than another layer. The layer(s) comprising a composition of the present invention can be any one or more of a core layer, an intermediate layer, or a cover layer.

#### Core Layer(s)

25 Cores of the golf balls formed according to the invention may be solid, semi-solid, hollow, fluid-, powder-, or gas-filled, and may be one-piece or multi-layered. Multilayer cores include a center, innermost portion, which may be solid, semi-solid, hollow, fluid-, powder-, or gas-filled, surrounded by at least one outer core layer. The outer core layer may be solid, or it may be a wound layer formed of a tensioned elastomeric material. For purposes of the present disclosure, the term "semi-solid" refers to a paste, a gel, or the like.

30 In a particular embodiment, the present invention provides a golf ball having an innermost core layer formed from a heterogeneous composition of the present invention. In another particular embodiment, the present invention provides a golf ball having an outer core layer formed from a heterogeneous composition of the present invention. In another particular embodiment, the present invention provides a golf ball having an intermediate core layer formed from a heterogeneous composition of the present invention.

35 Golf ball cores of the present invention may include one or more layers formed from a suitable material other than a heterogeneous composition of the present invention. Suitable core materials include, but are not limited to, thermoset materials, such as styrene butadiene rubber, polybutadiene, synthetic or natural polyisoprene, and trans-polyisoprene;

## 11

thermoplastics, such as ionomer resins, polyamides and polyesters; and thermoplastic and thermoset polyurethane and polyureas.

## Intermediate Layer(s)

When the golf ball of the present invention includes one or more intermediate layers, i.e., layer(s) disposed between the core and the cover of a golf ball, each intermediate layer can include any materials known to those of ordinary skill in the art including thermoplastic and thermosetting materials.

In one embodiment, the present invention provides a golf ball having one or more intermediate layers formed from a heterogeneous composition of the present invention.

Also suitable for forming intermediate layer(s) are the compositions disclosed above for forming core layers.

A moisture vapor barrier layer is optionally employed between the core and the cover. Moisture vapor barrier layers are further disclosed, for example, in U.S. Pat. Nos. 6,632,147, 6,838,028, 6,932,720, 7,004,854, and 7,182,702, and U.S. Patent Application Publication Nos. 2003/0069082, 2003/0069085, 2003/0130062, 2004/0147344, 2004/0185963, 2006/0068938, 2006/0128505 and 2007/0129172, the entire disclosures of which are hereby incorporated herein by reference.

## Cover

Golf ball covers of the present invention include single, dual, and multilayer covers. Dual and multilayer covers have an inner cover layer and an outer cover layer, and multilayer covers additionally have at least one intermediate cover layer disposed between the inner cover layer and the outer cover layer.

In a particular embodiment, the present invention provides a golf ball having an outermost cover layer formed from a heterogeneous composition of the present invention. In another particular embodiment, the present invention provides a golf ball having an inner cover layer formed from a heterogeneous composition of the present invention. In another particular embodiment, the present invention provides a golf ball having an intermediate cover layer formed from a heterogeneous composition of the present invention.

Golf ball covers of the present invention may include one or more layers formed from a suitable material other than a heterogeneous composition of the present invention. The cover material is preferably a tough, cut-resistant material, selected based on the desired performance characteristics.

Suitable cover materials for the golf balls disclosed herein include, but are not limited to, polyurethanes, polyureas, and hybrids of polyurethane and polyurea; ionomer resins and blends thereof (e.g., Surlyn® ionomer resins and DuPont® HPF 1000 and HPF 2000 highly neutralized ionomers, commercially available from E. I. du Pont de Nemours and Company; Iotek® ionomers, commercially available from ExxonMobil Chemical Company; Amplify® 10 ionomers of ethylene acrylic acid copolymers, commercially available from The Dow Chemical Company; and Clarix® ionomer resins, commercially available from A. Schulman Inc.); polyisoprene; polyoctenamer, such as Vestenamer® polyoctenamer, commercially available from Evonik Industries;

polyethylene, including, for example, low density polyethylene, linear low density polyethylene, and high density polyethylene; polypropylene; rubber-toughened olefin polymers; non-ionomeric acid copolymers, e.g., ethylene (meth) acrylic acid; plastomers; flexomers; styrene/butadiene/styrene block copolymers; polybutadiene; styrene butadiene rubber; ethylene propylene rubber; ethylene propylene diene rubber; styrene/ethylene-butylene/styrene block copolymers; dynamically vulcanized elastomers; ethylene vinyl acetates; ethylene (meth)acrylates; polyvinyl chloride res-

## 12

ins; polyamides, amide-ester elastomers, and copolymers of ionomer and polyamide, including, for example, Pebax® thermoplastic polyether and polyester amides, commercially available from Arkema Inc; crosslinked trans-polyisoprene and blends thereof; polyester-based thermoplastic elastomers, such as Hytrel® polyester elastomers, commercially available from E. I. du Pont de Nemours and Company, and Riteflex® polyester elastomers, commercially available from Ticona; polyurethane-based thermoplastic elastomers, such as Elastollan®, commercially available from BASF; synthetic or natural vulcanized rubber; and combinations thereof.

Polyurethanes, polyureas, and polyurethane-polyurea hybrids (i.e., blends and copolymers of polyurethanes and polyureas) are particularly suitable for forming cover layers of the present invention. Suitable polyurethanes and polyureas are further disclosed, for example, in U.S. Pat. Nos. 5,334,673, 5,484,870, 6,506,851, 6,756,436, 6,835,794, 6,867,279, 6,960,630, and 7,105,623; U.S. Patent Application Publication No. 2009/0011868; and U.S. Patent Application No. 60/401,047, the entire disclosures of which are hereby incorporated herein by reference. Suitable polyurethane-urea cover materials include polyurethane/polyurea blends and copolymers comprising urethane and urea segments, as disclosed in U.S. Patent Application Publication No. 2007/0117923, the entire disclosure of which is hereby incorporated herein by reference.

Compositions comprising an ionomer or a blend of two or more ionomers are also particularly suitable for forming cover layers. Preferred ionomeric cover compositions include:

- (a) a composition comprising a “high acid ionomer” (i.e., having an acid content of greater than 16 wt %), such as Surlyn® 8150;
- (b) a composition comprising a high acid ionomer and a maleic anhydride-grafted non-ionomeric polymer (e.g., Fusabond® functionalized polymers). A particularly preferred blend of high acid ionomer and maleic anhydride-grafted polymer is a 84 wt %/16 wt % blend of Surlyn® 8150 and Fusabond®. Blends of high acid ionomers with maleic anhydride-grafted polymers are further disclosed, for example, in U.S. Pat. Nos. 6,992,135 and 6,677,401, the entire disclosures of which are hereby incorporated herein by reference;
- (c) a composition comprising a 50/45/5 blend of Surlyn® 8940/Surlyn® 9650/Nucrel® 960, preferably having a material hardness of from 80 to 85 Shore C;
- (d) a composition comprising a 50/25/25 blend of Surlyn® 8940/Surlyn® 9650/Surlyn® 9910, preferably having a material hardness of about 90 Shore C;
- (e) a composition comprising a 50/50 blend of Surlyn® 8940/Surlyn® 9650, preferably having a material hardness of about 86 Shore C;
- (f) a composition comprising a blend of Surlyn® 7940/Surlyn® 8940, optionally including a melt flow modifier;
- (g) a composition comprising a blend of a first high acid ionomer and a second high acid ionomer, wherein the first high acid ionomer is neutralized with a different cation than the second high acid ionomer (e.g., 50/50 blend of Surlyn® 8150 and Surlyn® 9150), optionally including one or more melt flow modifiers such as an ionomer, ethylene-acid polymer or ester polymer; and
- (h) a composition comprising a blend of a first high acid ionomer and a second high acid ionomer, wherein the first high acid ionomer is neutralized with a different cation than the second high acid ionomer, and from 0

to 10 wt % of an ethylene/acid/ester ionomer wherein the ethylene/acid/ester ionomer is neutralized with the same cation as either the first high acid ionomer or the second high acid ionomer or a different cation than the first and second high acid ionomers (e.g., a blend of 40-50 wt % Surlyn® 8150, 40-50 wt % Surlyn® 9120, and 0-10 wt % Surlyn® 6320).

Surlyn® 8150 and Surlyn® 8940 are different grades of E/MAA copolymer in which the acid groups have been partially neutralized with sodium ions. Surlyn® 9650, Surlyn® 9910, Surlyn® 9150, and Surlyn® 9120 are different grades of E/MAA copolymer in which the acid groups have been partially neutralized with zinc ions. Surlyn® 7940 is an E/MAA copolymer in which the acid groups have been partially neutralized with lithium ions. Surlyn® 6320 is a very low modulus magnesium ionomer with a medium acid content. Nucrel® 960 is an E/MAA copolymer resin nominally made with 15 wt % methacrylic acid. Surlyn® ionomers, Fusabond® polymers, and Nucrel® copolymers are commercially available from E. I. du Pont de Nemours and Company.

Ionomeric cover compositions can be blended with non-ionic thermoplastic resins, such as polyurethane, poly-ether-ester, poly-amide-ether, polyether-urea, thermoplastic polyether block amides (e.g., Pebax® polyether and poly-ester amides, commercially available from Arkema Inc.), styrene-butadiene-styrene block copolymers, styrene(ethylene-butylene)styrene block copolymers, polyamides, polyesters, polyolefins (e.g., polyethylene, polypropylene, ethylene-propylene copolymers, polyethylene-(meth)acrylate, polyethylene-(meth)acrylic acid, functionalized polymers with maleic anhydride grafting, Fusabond® functionalized polymers commercially available from E. I. du Pont de Nemours and Company, functionalized polymers with epoxidation, elastomers (e.g., ethylene propylene diene monomer rubber, metallocene-catalyzed polyolefin) and ground powders of thermoset elastomers.

Ionomer golf ball cover compositions may include a flow modifier, such as, but not limited to, acid copolymer resins (e.g., Nucrel® acid copolymer resins, and particularly Nucrel® 960, commercially available from E. I. du Pont de Nemours and Company), performance additives (e.g., A-C® performance additives, particularly A-C® low molecular weight ionomers and copolymers, A-C® oxidized polyethylenes, and A-C® ethylene vinyl acetate waxes, commercially available from Honeywell International Inc.), fatty acid amides (e.g., ethylene bis-stearamide and ethylene bis-oleamide), fatty acids and salts thereof.

Suitable ionomeric cover materials are further disclosed, for example, in U.S. Pat. Nos. 6,653,382, 6,756,436, 6,894, 098, 6,919,393, and 6,953,820, the entire disclosures of which are hereby incorporated by reference.

Suitable cover materials and constructions also include, but are not limited to, those disclosed in U.S. Patent Application Publication No. 2005/0164810, U.S. Pat. Nos. 5,919, 100, 6,117,025, 6,767,940, and 6,960,630, and PCT Publications WO00/23519 and WO00/29129, the entire disclosures of which are hereby incorporated herein by reference.

#### Component Dimensions

Dimensions of golf ball components, i.e., thickness and diameter, may vary depending on the desired properties. For the purposes of the invention, any layer thickness may be employed.

The present invention relates to golf balls of any size. While USGA specifications limit the size of a competition golf ball to more than 1.68 inches in diameter, golf balls of

any size can be used for leisure golf play. The preferred diameter of the golf balls is from about 1.68 inches to about 1.8 inches. The more preferred diameter is from about 1.68 inches to about 1.76 inches. A diameter of from about 1.68 inches to about 1.74 inches is most preferred, however diameters anywhere in the range of from 1.7 to about 1.95 inches can be used.

Golf ball cores of the present invention include single, dual, and multilayer cores, and preferably have an overall diameter within the range having a lower limit of 0.75 inches or 1 inch or 1.25 inches or 1.4 inches and an upper limit of 1.55 inches or 1.6 inches or 1.62 inches or 1.63 inches. In a particular embodiment, the golf ball comprises a core and a cover, wherein the core is a solid, single layer having a diameter within a range having a lower limit of 0.750 or 1.00 or 1.10 or 1.15 or 1.20 or 1.25 or 1.30 or 1.40 or 1.50 or 1.53 or 1.55 inches and an upper limit of 1.55 or 1.60 or 1.62 or 1.63 or 1.65 inches. In another particular embodiment, the golf ball comprises a core and a cover, wherein the core comprises an inner core layer and an outer core layer, the inner core layer having a diameter within a range having a lower limit of 0.500 or 0.750 or 0.900 or 0.950 or 1.000 inches and an upper limit of 1.100 or 1.200 or 1.250 or 1.400 or 1.550 or 1.570 or 1.580 inches, and the outer core having a thickness within the range having a lower limit of 0.020 or 0.025 or 0.032 or 0.050 or 0.100 or 0.200 inches and an upper limit of 0.310 or 0.440 or 0.500 or 0.560 or 0.800 inches.

When present in a golf ball of the present invention, each intermediate layer has a thickness within a range having a lower limit of 0.002 or 0.010 or 0.020 or 0.025 or 0.030 inches and an upper limit of 0.035 or 0.040 or 0.045 or 0.050 or 0.060 or 0.090 or 0.100 or 0.150 or 0.200 inches. The total thickness of intermediate core layer(s) in golf balls of the present invention is preferably within the range having a lower limit of 0.020 or 0.0250 or 0.032 inches and an upper limit of 0.150 or 0.220 or 0.28 inches.

Golf ball covers of the present invention include single, dual, and multilayer covers, and preferably have an overall thickness within the range having a lower limit of 0.01 inches or 0.02 inches or 0.025 inches or 0.03 inches or 0.04 inches or 0.045 inches or 0.05 inches or 0.06 inches and an upper limit of 0.07 inches or 0.075 inches or 0.08 inches or 0.09 inches or 0.1 inches or 0.15 inches or 0.2 inches or 0.3 inches or 0.5 inches. Dual and multilayer covers have an inner cover layer and an outer cover layer, and multilayer covers additionally have at least one intermediate cover layer disposed between the inner cover layer and the outer cover layer. In a particular embodiment, the cover is a single layer having a thickness within a range having a lower limit of 0.020 or 0.025 or 0.030 inches and an upper limit of 0.030 or 0.040 or 0.045 or 0.050 or 0.070 or 0.100 or 0.120 or 0.150 or 0.350 or 0.400 or inches. In another particular embodiment, the cover comprises an inner cover layer and an outer cover layer, the inner cover having a thickness within a range having a lower limit of 0.010 or 0.020 or 0.025 or 0.030 inches and an upper limit of 0.035 or 0.040 or 0.050 or 0.150 or 0.200 inches, and the outer cover having a thickness within a range having a lower limit of 0.010 or 0.020 or 0.025 or 0.030 inches and an upper limit of 0.035 or 0.040 or 0.050 inches.

The golf balls of the present invention may be painted, coated, or surface treated for further benefits.

When numerical lower limits and numerical upper limits are set forth herein, it is contemplated that any combination of these values may be used.

## 15

All patents, publications, test procedures, and other references cited herein, including priority documents, are fully incorporated by reference to the extent such disclosure is not inconsistent with this invention and for all jurisdictions in which such incorporation is permitted.

While the illustrative embodiments of the invention have been described with particularity, it will be understood that various other modifications will be apparent to and can be readily made by those of ordinary skill in the art without departing from the spirit and scope of the invention. Accordingly, it is not intended that the scope of the claims appended hereto be limited to the examples and descriptions set forth herein, but rather that the claims be construed as encompassing all of the features of patentable novelty which reside in the present invention, including all features which would be treated as equivalents thereof by those of ordinary skill in the art to which the invention pertains.

What is claimed is:

1. A golf ball comprising a layer formed from a heterogeneous composition, the heterogeneous composition comprising:

a matrix formed from a thermosetting polymer composition, and  
discrete particles dispersed within the matrix, wherein the  
discrete particles are formed from a crosslinked rubber  
composition having a Shore A hardness of 50 or less.

## 16

2. The golf ball of claim 1, wherein the discrete particles are present in the heterogeneous composition in an amount of 60 wt % or greater, based on the total weight of the heterogeneous composition.

3. A golf ball comprising a layer formed from a heterogeneous composition, the heterogeneous composition comprising:

a matrix formed from a thermosetting polymer composition, and  
discrete particles dispersed within the matrix, wherein the  
discrete particles are formed from a crosslinked rubber  
composition having a Shore A hardness of 50 or less and comprising a peroxide initiator and from 0 to 5 phr of a coagent.

4. The golf ball of claim 3, wherein the discrete particle composition is substantially free of a coagent.

5. The golf ball of claim 3, wherein the peroxide initiator is present in the discrete particle composition in an amount of 10 phr or less.

6. The golf ball of claim 3, wherein the peroxide initiator is present in the discrete particle composition in an amount of 5 phr or less.

7. The golf ball of claim 3, wherein the discrete particles are present in the heterogeneous composition in an amount of 60 wt % or greater, based on the total weight of the heterogeneous composition.

\* \* \* \* \*